# EUROPEAN PATENT SPECIFICATION

(11) **EP 2 081 695 B1**
(45) Date of publication and mention of the grant of the patent: **02.12.2015**
(21) Application number: 07838833.7
(22) Date of filing: 25.09.2007
(51) Int. Cl.: B05D 7/00

(54) **PROCESS FOR THE PRODUCTION OF MULTI-LAYER COATINGS**
VERFAHREN ZUR HERSTELLUNG VON MEHRSCHICHTIGEN ÜBERZÜGEN
PROCESSUS POUR LA PRODUCTION DE REVÊTEMENTS MULTICOUCHES

(30) Priority: 25.10.2006 US 854269 P
(43) Date of publication of application: 29.07.2009
(73) Proprietor: Coatings Foreign IP Co. LLC, Wilmington, DE 19801 (US)
(72) Inventor: TIEGS, Frank-Peter, 42283 Wuppertal (DE); GEORGIADIS, Michael, 42389 Wuppertal (DE); CHILLA, Marc, 45549 Sprockhoevel (DE)
(74) Representative: Maiwald Patentanwalts GmbH
(86) International application number: PCT/US2007/020704
(87) International publication number: WO 2008/051346

(56) References cited:
- WO-A-2007/041228
- WO-A-2007/146386
- US-A1- 2006 008 588
- US-A1- 2006 068 116
- US-A1- 2006 134 334

## Description

### Field of the Invention

The invention relates to a process for the production of multi-layer coatings.

### Background of the Invention

Automotive coatings generally comprise a separately baked electrode position coating (EDC) primer, a separately baked primer surfacer layer (filler layer) applied thereto and a top coat applied thereto comprising a wet-on-wet applied color- and/or special effect-imparting base coat layer and a protective, gloss-imparting clear coat layer. The total primer surfacer plus base coat layer thickness is generally 30 to 60 µm, in case of metallic color shades (color tones) more in the lower range of 30 to 45 µm.

Processes are known from WO 97/47401 and U.S. 5,976,343 for the production of decorative multi-layer coatings, which processes allow for the elimination of the application and separate baking of a primer surfacer layer which, of course, reduces coating material consumption and total layer thickness. In these processes, a multi-layer coating structure comprising a first, modified water-borne base coat, a second, unmodified water-borne base coat and a clear coat is applied by a wet-on-wet-on-wet process comprising the joint curing of these three coating layers that are applied to a baked EDC primer. In practice, these processes use two base coat layers that allow for markedly lower total layer thickness by approximately 15 to 25 µm, than that of a conventional primer surfacer and base coat. The modified water-borne base coat is produced in these processes from an unmodified water-borne base coat by mixing with an admixture component. The modified water-borne base coat replaces a conventional primer surfacer. WO 97/47401 recommends as an admixture component, the addition of polyisocyanate crosslinking agent, while U.S. 5,976,343 describes the addition of polyurethane resin.

A weakness of the processes known from WO 97/47401 and U.S. 5,976,343 is that it is not straightforwardly possible to produce multi-layer coatings in certain color shades ("problematic color shades"). Color shades which are problematic with regard to the production of multi-layer coatings without primer surfacer layer are those color shades with low hiding power. Such color shades are problematic because the substrate shows through the base coat layer produced from modified and unmodified water-borne base coat. In the case of substrates with a nonuniform color shade and/or due to fluctuations in film thickness (nonuniform distribution of film thickness on the substrate) of the base coat layer, nonuniformity of color shade is perceived. Bake-cured EDC primer coatings in particular are examples of problematic substrates which are nonuniform in color shade, because they often suffer from severe local discoloration as the result of localized differences in object temperature during bake curing. The problematic color shades are to be found both among solid color shades (plain color shades, single-tone color shades; generally independent of observation angle; pigment content without special effect pigments) and special effect color shades.

The problem could be solved by applying the modified and/or the unmodified water-borne base coat in an overall higher, opaque layer thickness. However, this would be a backward technological step in the direction of high total film thickness, and the high, opaque film thickness would have to be built up in several applications, which would not be of assistance in ensuring a maximally economic coating process.

US 2006/068116 A1 describes a process producing multilayer coatings in light metallic color shades comprising three successive steps.

WO 2007/041228 and WO 2007/016386 A, both documents under Article 54(3) EPC, also describe processes for the production of multilayer coatings comprising several successive steps.

Raising the pigment content of the unmodified water-borne base coat is limited, on the one hand, by the critical pigment volume concentration, but is in general also not feasible with regard to the required technological properties of the finished coating.

### Summary of the Invention

The invention is directed to a process for the production of multi-layer coatings in A' color shades, comprising the successive steps:
1) applying a two-layered base coat layer in a total process film thickness in the range from 10 to 35 µm to a substrate provided with an EDC primer,
2) applying a clear coat layer onto the base coat layer,
3) jointly curing the base coat and clear coat layers,
wherein step 1) comprises (i) mixing 100 pbv of an unmodified water-borne base coat A having a color shade A' and having a black/white opacity of >25 µm and 1 to 400 pbv of an unmodified water-borne base coat B having a color shade B' to form an unmodified water-borne base coat AB, (ii) mixing the unmodified water-borne base coat AB with a pigment-free admixture component to form a modified water-borne base coat modAB, (iii) applying the first layer of the two-layered base coat layer from the modified water-borne base coat modAB and (iv) applying the second layer of the two-layered base coat layer from the unmodified water-borne base coat A,
wherein the pigment-free admixture component is a composition with a solids content of 29 to 95 wt.% consisting of a resin solids content plus possible nonvolatile additives, said resin solids content consisting of polyisocyanate(s),
wherein the admixture component is mixed into the unmodified water-borne base coat AB in a ratio by weight of 0.2 to 1 parts of polyisocyanate : 1 part of resin solids of the unmodified water-borne base coat AB, and
wherein the pigment content of the unmodified water-borne base coat B is made such that the multi-layer coating achieved after step 3) achieves color shade consistency from in each case at least 80% of the individual process film thickness both of the layer applied from the modified water-borne base coat modAB and of the layer applied from the unmodified water-borne base coat A.

### Detailed Description of the Embodiments

The film thicknesses indicated in the description and in the claims for coating layers refer in each case to dry film thicknesses. In the description and the claims the term "process film thickness" is used. The meaning of this term will be explained hereinbelow.

The term "black/white opacity" is used in the description and the claims. It refers to the dry coating thickness of a coating composition wherein the contrast between the black and white fields of a black and white chart coated with the coating composition is no longer visually discernible (mean coating thickness value determined on the basis of evaluation by 5 independent individuals). Following ISO 6504-3:2006 (E), method B, in order to determine this coating thickness, the coating composition of which the black/white opacity is to be investigated may be applied in a wedge shape onto a black and white chart and dried or hardened.

The term "pigment content" used in the description and in the claims means the sum of all the pigments contained in a coating composition without fillers (extenders). The term "pigments" is used here as in DIN 55944 and covers, in addition to special effect pigments, inorganic white, colored and black pigments and organic colored and black pigments. At the same time, therefore, DIN 55944 distinguishes between pigments and fillers.

The description and the claims mention "one or more binders C". This serves to distinguish between the binder(s) of the unmodified water-borne base coats A, B and AB and the binder(s) C of the pigment-free admixture component I.

The phrase used in the description and the claims "color shade consistency of the multi-layer coating from in each case at least 80% of the individual process film thickness both of the layer applied from the modified water-borne base coat modAB and of the layer applied from the unmodified water-borne base coat A" means that the color difference delta E [delta E can be determined by goniospectrophotometric colorimetry and it equals the square root of (delta L² + delta C² + delta h²); L, C, h = lightness, chroma, hue] between multi-layer coatings to be compared and applied from modified water-borne base coat modAB, unmodified water-borne base coat A and clear coat is sufficiently small if the base coat layers applied both from the modified water-borne base coat modAB and from the unmodified water-borne base coat A have each been applied to 80% or more of the individual process film thickness. In the case of solid color shades, delta E values of < 0.4 determined at an illumination angle of 45° to the perpendicular and an observation angle of 45° relative to the specular reflection are sufficiently small and thus represent color shade consistency in the above sense. In the case of special effect color shades (dependent on observation angle; pigment content comprises at least one special effect-imparting pigment) delta E values are sufficiently small if the delta E values, when determined at an illumination angle of 45° to the perpendicular and at observation angles of 15, 25, 45, 75 and 110° relative to the specular reflection are in each case < 2.

In goniospectrophotometric colorimetry the reflectance curves of visible light in the range from, for example, 380 to 800 nm of a coated surface are determined at one or more different observation angles. The reflectance curves may, for example, be determined at 5 observation angles, for example at 15, 25, 45, 75 and 110° relative to the specular reflection. The reflectance curves may be used as the basis for calculating the conventional CIELab system colorimetric parameters L* (lightness), a* (red-green value), b* (yellow-blue value) and further also C* (chroma) and h* (hue) (c.f. DIN 6174) or these values are directly output from the measuring instrument. The reflectance curves may be determined using any conventional colorimeters known to the person skilled in the art, for example, the X-Rite MA 68 II instrument sold by the company X-Rite. In the process according to the invention conventional substrates provided with an EDC primer, preferably a cathodic electrodeposition (CED) coating, are coated. In particular, the substrates are automotive bodies or automotive body parts. The production of substrates provided with an EDC primer is known to the person skilled in the art.

In step 1) of the process according to the invention, the substrates having an EDC primer are provided, with a base coat layer in a total process film thickness in the range from 10 to 35 µm. This base coat layer is applied in two layers, i.e., a first layer having an individual process film thickness in the range from, for example, 5 to 25 µm of a modified water-borne base coat modAB produced by mixing an unmodified water-borne base coat AB with a pigment-free admixture component is applied and a subsequent second layer in an individual process film thickness below black/white opacity, for example, in the range from 3 to 20 µm of the unmodified water-borne base coat A then is applied. The total process film thickness of the base coat layer is dependent inter alia on color shade. Car manufacturers' requirements for base coat film thickness are expressed in the so-called process film thickness (average film thickness which is desired over the entire body in the automotive original coating process), which depends on the individual color shade, on technological properties to be achieved (e.g., stone chip resistance) and on an economic application of the relevant water-borne base coat, i.e., in as thin a film as possible. The total base coat process film thickness lies in the range from 10 to 35 µm and is the sum of, for example, 5 to 25 µm of the modified water-borne base coat modAB plus, for example, 3 to 20 µm of the unmodified water-borne base coat A. Such film thicknesses for base coats meet the requirements for coating the relevant substrates, for example, automotive bodies. In particular, this means that a specific value within this range from 10 to 35 µm represents the specific total process film thickness for a particular base coat, for example, a base coat of a particular color shade. Said specific total process film thickness is here composed of the sum of the specific individual process film thickness, lying within the range of, for example, 5 to 25 µm, of the corresponding modified water-borne base coat modAB and the specific individual process film thickness, lying within the range of, for example, 3 to 20 µm of the corresponding unmodified water-borne base coat A.

In the present invention a distinction is drawn between (i) unmodified water-borne base coats A, B and AB and (ii) modified water-borne base coats modAB. Whereas the unmodified water-borne base coats A are water-borne base coats with problematic color shades and having low hiding power, the unmodified water-borne base coats B are water-borne base coats with unproblematic color shades and having sufficient hiding power.

The color shades of a coating applied from an unmodified water-borne base coat A in opaque film thickness and of a corresponding multi-layer coating prepared according to the process of the invention are so close to each other that an observer virtually cannot perceive a difference between the color shades. Therefore, in the present description and the claims, the color shades of the unmodified water-borne base coats A and of coatings applied thereof in opaque film thickness are called color shades A'. The color shades of the corresponding multi-layer coatings prepared according to the process of the invention are also called color shades A'. Accordingly, the color shades of the unmodified water-borne base coats B and of coatings applied thereof in opaque film thickness are called color shades B'.

The unmodified water-borne base coats AB may be produced by mixing 100 pbv of unmodified water-borne base coat A with 1 to 400 pbv, for example, 1 to 50 pbv of an unmodified water-borne base coat B. The unmodified water-borne base coat B to be mixed with the unmodified water-borne base coat A may be one individual water-borne base coat B or a mixture of two or more different unmodified water-borne base coats B; preferably it is one individual-water-borne base coat B. Usually the mixing ratio will be 100 pbv of unmodified water-borne base coat A : 1 to 50 pbv of unmodified water-borne base coat B. A mixing ratio of 100 pbv of unmodified water-borne base coat A : more than 50 to 400 pbv of unmodified water-borne base coat B applies in particular in case the unmodified water-borne base coat B is a light-colored or even a white unmodified water-borne base coat.

The modified water-borne base coats modAB may be produced by (i) mixing the unmodified water-borne base coats AB with the pigment-free admixture component I in a ratio by weight of 0.1 to 1 parts of binder(s) C : 1 part of resin solids of the unmodified water-borne base coat AB or by (ii) mixing the unmodified water-borne base coats AB with the pigment-free admixture component II in a ratio by weight of 0.2 to 1 parts of polyisocyanate : 1 part of resin solids of the unmodified water-borne base coat AB.

In principle there is no restriction regarding the mixing sequence provided the stated volume and weight ratios are met. To avoid misunderstandings, the phrase "a modified water-borne base coat modAB produced by mixing an unmodified water-borne base coat AB with a pigment-free admixture component" shall not be understood to rule out another mixing sequence. In other words, it is possible to mix the unmodified water-borne base coats A and B first and then to mix the resulting unmodified water-borne base coat AB with the pigment-free admixture component I or II; especially in case of an admixture component II this is the preferred mixing sequence. However, it is also possible to mix the unmodified water-borne base coat A or B with the pigment-free admixture component I or II first and then to mix the resulting mixture with the unmodified water-borne base coat B or A; this mixing sequence corresponds to an insitu production of an unmodified water-borne base coat AB. It is also possible to mix the unmodified water-borne base coats A and B and the pigment-free admixture component I or II simultaneously.

The unmodified water-borne base coats A and B must be chemically compatible with each other, i.e. miscible with each other without problems, for example, without formation of coagulate or precipitate. Whereas this is generally guaranteed in case unmodified water-borne base coats A and B are supplied by the same paint manufacturer, it is necessary to ensure such compatibility in case there is more than one supplier for the unmodified water-borne base coats A and B. The unmodified water-borne base coats A and B to be mixed should not differ from each other too much in viscosity to allow for easy mixing. For example, the difference in viscosity should not exceed 50 mPa·s at a shear rate of 1000 s⁻¹ at 20°C.

The unmodified water-borne base coats A, B and AB are aqueous coating compositions having a ratio by weight of pigment content to resin solids content of, for example, 0.05 : 1 to 1 : 1. In addition to water, pigment(s), a resin solids content, which comprises binder(s), optionally, paste resin(s) and optionally, cross-linking agent(s), optionally, filler(s) and optionally, organic solvent(s), the unmodified water-borne base coats A, B and AB contain in general also conventional additive(s).

The unmodified water-borne base coats A, B and AB contain ionically and/or non-ionically stabilized binder systems. In case of ionic stabilization anionic stabilization is preferred. Anionic stabilization is preferably achieved by at least partially neutralized carboxyl groups in the binder, while non-ionic stabilization is preferably achieved by lateral or terminal polyethylene oxide units in the binder. The unmodified water-borne base coats A, B and AB may be physically drying or crosslinkable by formation of covalent bonds. The crosslinkable unmodified water-borne base coats A, B and AB forming covalent bonds may be self- or externally crosslinkable systems.

The unmodified water-borne base coats A, B and AB contain one or more conventional film-forming binders. They may optionally also contain crosslinking agents if the binders are not self-crosslinkable or physically drying. Examples of film-forming binders, which may be used, are conventional polyester, polyurethane, (meth)acrylic copolymer and/or hybrid resins derived from these classes of resin. Selection of the optionally contained crosslinking agents depends, in a manner familiar to the person skilled in the art, on the functionality of the binders, i.e., the crosslinking agents are selected in such a way that they exhibit a reactive functionality complementary to the functionality of the binders. Examples of such complementary functionalities between binder and crosslinking agent are: carboxyl/epoxy, hydroxyl/methylol ether and/or methylol (methylol ether and/or methylol preferably, as crosslinkable groups of aminoplast resins, in particular, melamine resins).

The term "polyurethane resin" as used in the present invention does not rule out that the polyurethane resin in question may also contain groups other than urethane groups in the polymer backbone, such as, in particular, ester groups and/or urea groups. Instead, the term "polyurethane resin" of course, also in particular, includes polyurethane resins which contain polyester polyol building blocks and/or urea groups, wherein the latter may, for example, be formed by the reaction of isocyanate groups with water and/or polyamine.

If the process according to the invention is performed with a pigment-free admixture component II, it is preferred to work with unmodified water-borne base coats AB which comprise a resin solids content comprising one or more hydroxyl-functional binders. Here, the hydroxyl value of the resin solids content of the unmodified water-borne base coat AB is, for example, in the range of from 10 to 150 mg KOH/g, the NCO/OH molar ratio in the modified water-borne base coat modAB is, for example, 0.5 : 1 to 25 : 1. However, in the case of unmodified water-borne base coats AB with a low-hydroxyl or hydroxyl-free resin solids content, higher NCO/OH molar ratios may also arise in the corresponding modified water-borne base coats modAB. For example, the NCO/OH molar ratios may even extend towards infinity. In such cases, the polyisocyanate in the modified water-borne base coat modAB is consumed by reaction with other constituents, which are reactive in relation to isocyanate groups, for example, with water, hydroxyl-functional solvents and/or with functional groups of binders which are reactive with isocyanate and are different from hydroxyl groups.

The unmodified water-borne base coats A, B and AB contain conventional pigments, for example, special effect pigments and/or pigments selected from among white, colored and black pigments. Examples of special effect pigments are conventional pigments which impart to a coating color flop and/or lightness flop dependent on the observation angle, such as, non-leafing metal pigments, for example, of aluminum, copper or other metals, interference pigments, such as, for example, metal oxide-coated metal pigments, for example, iron oxide-coated aluminum, coated mica, such as, for example, titanium dioxide-coated mica, graphite effect-imparting pigments, iron oxide in flake form, liquid crystal pigments, coated aluminum oxide pigments, coated silicon dioxide pigments.

Examples of white, colored and black pigments are the conventional inorganic or organic pigments known to the person skilled in the art, such as, for example, titanium dioxide, iron oxide pigments, carbon black, azo pigments, phthalocyanine pigments, quinacridone pigments, pyrrolopyrrole pigments, perylene pigments.

The unmodified water-borne base coats A, B and AB may also contain fillers, for example, in proportions of 0 to 30 wt.% relative to the resin solids content. The fillers do not constitute part of the pigment content of the unmodified water-borne base coats A, B and AB. Examples are barium sulfate, kaolin, talcum, silicon dioxide, layered silicates and any mixtures thereof.

The special effect pigments are generally initially introduced in the form of a conventional commercial aqueous or non-aqueous paste, optionally, combined with preferably water-dilutable organic solvents and additives and then mixed with aqueous binder. Pulverulent special-effect pigments may first be processed with preferably water-dilutable organic solvents and additives to yield a paste.

White, colored and black pigments and/or fillers may, for example, be ground in a proportion of the aqueous binder. Grinding may preferably also take place in a special aqueous paste resin. Grinding may be performed in conventional assemblies known to the person skilled in the art. The formulation is then completed with the remaining proportion of the aqueous binder or of the aqueous paste resin.
The unmodified water-borne base coats A, B and AB may contain conventional additives in conventional quantities, for example, of 0.1 to 5 wt.%, relative to the solids content thereof. Examples are antifoaming agents, wetting agents, adhesion promoters, catalysts, levelling agents, anticratering agents, thickeners and light stabilizers.
The water content of the unmodified water-borne base coats A, B and AB is, for example, 60 to 90 wt.%.

The unmodified water-borne base coats A, B and AB may contain conventional organic solvents, for example, in a proportion of preferably less than 20 wt.%, particularly preferably, less than 15 wt.%. Examples of such solvents are mono- or polyhydric alcohols, for example, propanol, butanol, hexanol; glycol ethers or esters, for example, diethylene glycol di-C1-C6-alkyl ether, dipropylene glycol di-C1-C6-alkyl ether, ethoxypropanol, ethylene glycol monobutyl ether; glycols, for example, ethylene glycol and/or propylene glycol, and the di- or trimers thereof; N-alkylpyrrolidone, such as, for example, N-methylpyrrolidone; ketones, such as, methyl ethyl ketone, acetone, cyclohexanone; aromatic or aliphatic hydrocarbons, for example, toluene, xylene or linear or branched aliphatic C6-C12 hydrocarbons.

The unmodified water-borne base coats A, B and AB have solids contents of, for example, 10 to 40 wt.%, preferably, of 15 to 30 wt.%. The unmodified water-borne base coats A have a black/white opacity of >25 µm, i.e. they are water-borne base coats with problematic color shades and having low hiding power. They comprise pigments which according to the kind and/or quantity thereof allow only for a low hiding power. Examples are in particular unmodified water-borne base coats A with certain, in particular luminous blue, red, yellow or orange color shades which are especially distinguished by elevated brilliance and color purity. They may comprise solid color shades or special effect color shades, such as mica or metallic color shades.

The unmodified water-borne base coats A in particular comprise those which, despite their black/white opacity of >25 µm, are non-critical with regard to UV transmission, i.e., they comprise water-borne base coats which are distinguished in that UV light corresponding to a UV transmission of less than 0.1% in the wavelength range of from 280 to 380 nm, of less than 0.5% in the wavelength range of from 380 to 400 nm and of less than 1 % in the wavelength range of from 400 to 450 nm may penetrate through a base coat layer applied in the process film thickness and (i) consisting of a relevant unmodified water-borne base coat A mixed with the pigment-free admixture component I in a ratio by weight of 0.1 to 1 parts of binder(s) C : 1 part of resin solids of the unmodified water-borne base coat A and the corresponding unmodified water-borne base coat A or (ii) consisting of a relevant unmodified water-borne base coat A mixed with the pigment-free admixture component II in a ratio by weight of 0.2 to 1 parts of polyisocyanate : 1 part of resin solids of the unmodified water-borne base coat A and the corresponding unmodified water-borne base coat A. In other words, those unmodified water-borne base coats A have levels of pigmentation (ratio by weight of pigment content to resin solids content) and/or such pigment contents that, by virtue of the type and proportion of the constituent pigments, UV light corresponding to a UV transmission of less than 0.1 % in the wavelength range of from 280 to 380 nm, of less than 0.5% in the wavelength range of from 380 to 400 nm and of less than 1 % in the wavelength range of from 400 to 450 nm may penetrate through a base coat layer applied in the process film thickness and (i) consisting of a relevant unmodified water-borne base coat A mixed with the pigment-free admixture component I in a ratio by weight of 0.1 to 1 parts of binder(s) C : 1 part of resin solids of the unmodified water-borne base coat A and the corresponding unmodified water-borne base coat A or (ii) consisting of a relevant unmodified water-borne base coat A mixed with the pigment-free admixture component II in a ratio by weight of 0.2 to 1 parts of polyisocyanate : 1 part of resin solids of the unmodified water-borne base coat A and the corresponding unmodified water-borne base coat A. In still other and more general words, those unmodified water-borne base coats A have levels of pigmentation and/or pigment contents with or with sufficient proportions of pigments which effectively reduce UV transmission. UV transmission may be measured by applying a corresponding coating structure of unmodified water-borne base coat A mixed with the pigment-free admixture component I or II and unmodified water-borne base coat A to a UV light-transmitting support, for example, a silica glass plate, and measuring the UV transmission in the corresponding wavelength range using a corresponding uncoated UV light-transmitting support as reference.

The unmodified water-borne base coats B are water-borne base coats with unproblematic color shades and having sufficient hiding power, i.e. they comprise pigments which according to the kind and/or quantity thereof allow for sufficient hiding power. Examples are in particular unmodified water-borne base coats B with certain, in particular white, black, dark blue or green color shades. They may comprise solid color shades or special effect color shades, such as mica or metallic color shades. Unmodified water-borne base coats B with a solid color shade are preferred, in particular in case they are to be mixed with an unmodified water-borne base coat A with a solid color shade.

The pigment content of the unmodified water-borne base coat B is made such that, with a given (particular) unmodified water-borne base coat A, a given specific total process film thickness (and in each case also specific individual process film thicknesses for the modified water-borne base coat modAB and for the unmodified water-borne base coat A), a given mixing ratio of unmodified water-borne base coat A and B in the corresponding aforementioned range, a given mixing ratio of pigment-free admixture component I or II and unmodified water-borne base coat AB in the corresponding aforementioned range, the multi-layer coating produced from the modified water-borne base coat modAB applied to at least 80% of the specific individual process film thickness, from the corresponding unmodified water-borne base coat A applied to at least 80% of the specific individual process film thickness and the clear coat achieves color shade consistency. In particular, the pigment content of the unmodified water-borne base coat B is selected by type (qualitative and quantitative composition of the pigments forming the pigment content) and quantity accordingly.

The pigment contents of unmodified water-borne base coats B in particular comprise hiding power imparting pigments. Pigments capable of providing hiding power are known to the skilled person developing color shades of coatings. Suitable pigment contents are, for example, those with elevated proportions of hiding power imparting pigments within the pigment composition, for example, with 30 or more wt.% of carbon black, 70 or more wt.% of titanium dioxide or 40 or more wt.% of phthalocyanine pigments.

In the first embodiment of the process according to the invention the modified water-borne base coat modAB is produced from the unmodified water-borne base coat AB by mixing with the pigment-free admixture component I in a ratio by weight of 0.1 to 1 parts, preferably of 0.1 to 0.5 parts of binder(s) C : 1 part of resin solids of the unmodified water-borne base coat AB.

The addition of the pigment-free admixture component I to the unmodified water-borne base coat AB imparts to the resultant modified water-borne base coat modAB technological properties, such as, for example, stone chip resistance, which are important to the finished multi-layer coating. It is moreover ensured in this manner that color-consistent multi-layer coatings in the desired color shade (color shade specified by a coated standard) are obtained.

The pigment-free admixture component I containing one or more binder(s) C is a composition with a solids content of 20 to 95 wt.%, in general, of 30 to 60 wt.%. The volatile content is formed, in addition to possible volatile additives, by water and/or organic solvent. The solids content itself consists of the resin solids content plus possible nonvolatile additives.

The resin solids content of the pigment-free admixture component I comprises one or more binders C and, optionally, one or more crosslinking agents, for example, blocked polyisocyanates, aminoplast resins, such as, for example, melamine resins. In general, the resin solids content consists to an extent of, for example, 70 to 100 wt.% of the at least one binder C plus 0 to 30 wt.% of at least one crosslinking agent, wherein the weight percentages add up to 100 wt.%.

The binder(s) C of the pigment-free admixture component I may comprise the same binders as in the unmodified water-borne base coats A, B or AB and/or binders which differ therefrom.

The binder(s) C are conventional water-dilutable, preferably anionically stabilized binders, for example, corresponding polyester, polyurethane, (meth)acrylic copolymer and/or hybrid resins derived from these classes of resin. Polyester and in particular polyurethane resins are preferred.

Apart from the groups which ensure water dilutability, such as, in particular carboxyl groups, the binders C may comprise functional groups which may be involved in a crosslinking reaction which optionally proceeds during the subsequent thermal curing of the modified water-borne base coat modAB; such crosslinking reactions are in particular addition and/or condensation reactions. The binders C may also be self-crosslinkable. Examples of binders' C functional groups are hydroxyl groups, blocked isocyanate groups and epoxy groups.

The pigment-free admixture component I generally comprises an aqueous composition; it then contains, for example, 20 to 70 wt.% water.

Irrespective of whether it is an aqueous or non-aqueous composition, the pigment-free admixture component I may contain one or more organic solvents, for example, in a total quantity of 5 to 70 wt.%. Examples of such solvents are mono- or polyhydric alcohols, for example, propanol, butanol, hexanol; glycol ethers or esters, for example, diethylene glycol C1-C6 dialkyl ethers, dipropylene glycol C1-C6 dialkyl ethers, ethoxypropanol, butylglycol; glycols, for example, ethylene glycol and/or propylene glycol, and the di- or trimers thereof; N-alkylpyrrolidones, for example N-methylpyrrolidone and ketones, for example, methyl ethyl ketone, acetone, cyclohexanone; aromatic or aliphatic hydrocarbons, for example, toluene, xylene, or linear or branched aliphatic C6-C12 hydrocarbons. The solvents are preferably water-dilutable.

In addition to the at least one binder C and the in each case optional constituents water and organic solvent, the pigment-free admixture component I may contain additives in proportions of in each case, for example, 0.1 to 4 wt.%, corresponding to a total quantity of in general no more than 6 wt.%. Examples of additives are defoamers, anticratering agents, wetting agents, neutralizing agents, light stabilizers and rheology control agents.

Further, the modified water-borne base coat modAB can be produced from the unmodified water-borne base coat AB by mixing with the pigment-free admixture component II in a ratio by weight of 0.2 to 1 parts, preferably of 0.2 to 0.8 parts of polyisocyanate : 1 part of resin solids of the unmodified water-borne base coat AB.

The addition of the pigment-free admixture component II to the unmodified water-borne base coat AB imparts to the resultant modified water-borne base coat technological properties, such as, for example, stone chip resistance, which are important to the finished multi-layer coating. It is moreover ensured in this manner that color-consistent multi-layer coatings in the desired color shade (color shade specified by a coated standard) are obtained.

The pigment-free admixture component II containing one or more polyisocyanates is a composition with a solids content of, for example, 20 to 95 wt.%, in general, of 40 to 80 wt.%. The volatile content is formed, in addition to possible volatile additives, by water and/or organic solvent. The solids content itself consists of the resin solids content and, optionally, plus nonvolatile additives.

The resin solids content of the pigment-free admixture component II comprises one or more polyisocyanates. In general, the resin solids content consists to an extent of 100 wt.% of polyisocyanate(s).

The term "polyisocyanate(s)" used in connection with the pigment-free admixture component II is not restricted to the meaning free polyisocyanate or free polyisocyanates, but instead also includes blocked polyisocyanate or blocked polyisocyanates. The polyisocyanate(s) contained in the pigment-free admixture component II accordingly comprise one or more free polyisocyanates, one or more blocked polyisocyanates or a combination of one or more free polyisocyanates and one or more blocked polyisocyanates. Free polyisocyanates are preferred. The polyisocyanates comprise di- and/or poly-isocyanates with aliphatically, cycloaliphatically, araliphatically and/or less preferably aromatically attached isocyanate groups.

The polyisocyanates are liquid at room temperature or are present as an organic solution; the polyisocyanates here exhibit at 23°C a viscosity of in general 0.5 to 2000 mPa·s. The isocyanate content of the polyisocyanates present in the form of free or latent (blocked, thermally redissociable) isocyanate groups is in general in a range from 2 to 25 wt.%, preferably, from 5 to 25 wt.% (calculated as NCO).

Examples of diisocyanates are hexamethylene diisocyanate, tetramethylxylylene diisocyanate, isophorone diisocyanate, dicyclohexylmethane diisocyanate, and cyclohexane diisocyanate.

Examples of polyisocyanates are those which contain heteroatoms in the residue linking the isocyanate groups. Examples of these are polyisocyanates which contain carbodiimide groups, allophanate groups, isocyanurate groups, uretidione groups, urethane groups, acylated urea groups or biuret groups. The polyisocyanates preferably have an isocyanate functionality higher than 2, such as, for example, polyisocyanates of the uretidione or isocyanurate type produced by di- or trimerization of the above-mentioned diisocyanates. Further examples are polyisocyanates produced by reaction of the above-mentioned diisocyanates with water and containing biuret groups or polyisocyanates produced by reaction with polyols and containing urethane groups.

Of particular suitability are, for example, "coating polyisocyanates" based on hexamethylene diisocyanate, isophorone diisocyanate or dicyclohexylmethane diisocyanate. "Coating polyisocyanates" based on these diisocyanates means the per se known biuret, urethane, uretidione and/or isocyanurate group-containing derivatives of these diisocyanates.

As already mentioned above, the polyisocyanates may be used in blocked form, though this is not preferred. They may be blocked with conventional blocking agents that can be de-blocked under the action of heat, for example, with alcohols, oximes, amines and/or CH-acidic compounds.

The blocked or preferably free polyisocyanates may be used in the pigment-free admixture component II as such or as a preparation containing water and/or organic solvent, wherein in the case of free polyisocyanate no water and no organic solvent with active hydrogen is used. It may be desirable, for example, for the polyisocyanates to be prediluted with a water-miscible organic solvent or solvent mixture. In this case, it is preferable to use solvents, which are inert relative to isocyanate groups, especially where the preferred free polyisocyanates are used. Examples are solvents which do not contain any active hydrogen, for example, ethers, such as, for example, diethylene glycol diethyl ether, dipropylene glycol dimethyl ether; glycol ether esters, such as, ethylene glycol monobutyl ether acetate, diethylene glycol monobutyl ether acetate, methoxypropyl acetate; and N-methylpyrrolidone.

Also suitable are hydrophilic polyisocyanates, which may be stabilized in the aqueous phase by a sufficient number of ionic groups and/or by terminal or lateral polyether chains. Hydrophilic polyisocyanates are sold as commercial products, for example, by Bayer under the name Bayhydur®.

When producing a preferred pigment-free admixture component II containing free polyisocyanate, it is expedient not only to avoid the deliberate addition of water, but also to perform processing with the most extensive possible, preferably complete, exclusion of water and in general also with the most extensive possible, preferably complete, exclusion of other substances reactive towards isocyanate groups, such as, for example, alcohols. Apart from selecting appropriate raw materials, it is additionally possible to work with water-binding auxiliaries. For example, water scavengers, such as, orthoesters may be added during production and storage of the pigment-free admixture component II containing free polyisocyanate.

The pigment-free admixture component II may, if it contains no free polyisocyanate, contain, for example, 20 to 70 wt.% water.

The pigment-free admixture component II may contain one or more organic solvents, for example, in a total quantity of 5 to 70 wt.%. The solvents are preferably water-dilutable. In the case of the preferred admixture components II containing free polyisocyanate, the solvents are those which are inert towards isocyanate groups. Examples of suitable solvents are ethers, such as, for example, diethylene glycol diethyl ether, dipropylene glycol dimethyl ether; glycol ether esters, such as, ethylene glycol monobutyl ether acetate, diethylene glycol monobutyl ether acetate, methoxypropyl acetate; and N-methylpyrrolidone.

In addition to the at least one polyisocyanate and in each case optional constituents water and organic solvent, the pigment-free admixture component II may contain additives in proportions of in each case, for example, 0.1 to 2 wt.%, corresponding a total quantity of in general no more than 5 wt.%. Examples of additives are the same as those already mentioned for the pigment-free admixture component I.

As already mentioned, in the process according to the invention, the substrates are provided with multi-layer coatings in A' color shades. Typically, the multi-layer coating process according to the invention is performed in an industrial coating facility, i.e. within a mass-production coating line. Generally, there are not only substrates to be provided with multi-layer coatings in A' color shades but also substrates to be provided with corresponding multi-layer coatings in B' color shades. Coating of the latter substrates is performed making use of unmodified water-borne base coats B and, in that case the unmodified water-borne base coats A and the unmodified water-borne base coats B together represent the color shade program selected for the substrates to be multi-layer coated. It is advantageous that the unmodified water-borne base coats B to be mixed with the unmodified water-borne base coats A can then be taken from the group of unmodified water-borne base coats B which represent the B' color shade program. In general the B' color shade program comprises two or more differently colored unmodified water-borne base coats B. This allows for the selection of an appropriate unmodified water-borne base coat B (one individual water-borne base coat B or a mixture of two or more different unmodified water-borne base coats B). In particular such selection may happen dependent on the color shade of the relevant unmodified water-borne base coat A to be mixed with.

As already mentioned, the unmodified water-borne base coats B comprise unmodified water-borne base coats with unproblematic color shades and having sufficient hiding power. Therefore, the process for the production of multi-layer coatings on substrates in B' color shades is different from the process according to the invention. Preferably, the process for the production of multi-layer coatings in B' color shades comprises the successive steps:
1) applying a base coat layer in a total process film thickness in the range from 10 to 35 µm to a substrate provided with an EDC primer,
2) applying a clear coat layer onto the base coat layer,
3) jointly curing the base coat and clear coat layers,
wherein the base coat layer is applied in a first layer and, optionally, in a second layer; the first layer comprises a modified water-borne base coat modB produced by mixing an unmodified water-borne base coat B having a color shade B' with a pigment-free admixture component and the optionally applied second layer comprises the unmodified water-borne base coat B,
wherein the pigment-free admixture component is selected from the group consisting of a pigment-free admixture component I and a pigment-free admixture component II, wherein admixture component I comprises one or more binders C, and being mixed into the unmodified water-borne base coat B in a ratio by weight of 0.1 to 1 parts of binder(s) C : 1 part of resin solids of the unmodified water-borne base coat B; and wherein admixture component II comprises one or more polyisocyanates, and being mixed into the unmodified water-borne base coat B in a ratio by weight of 0.2 to 1 parts of polyisocyanate : 1 part of resin solids of the unmodified water-borne base coat B.

In the process according to the invention, the unmodified water-borne base coats A, B and the pigment-free admixture component are mixed preferably on the user's premises, in particular shortly or immediately before application of the resultant modified water-borne base coat modAB. As already mentioned, there are various possibilities for the mixing sequence.

In the case of industrial coating facilities, the unmodified water-borne base coats A and B in each case of a different color shade are each conveyed in their own circulating line. The pigment-free admixture component to be added is preferably used in the form of a single general purpose admixture component, the one pigment-free admixture component likewise being guided in its own circulating line and automatically mixed with the respective unmodified water-borne base coats A and B using mixing technology conventional in industrial coating facilities, for example, a static mixer like a Kenics mixer. When applying water-borne base coat in a color shade program of n A' and m B' color shades, it is therefore not necessary to provide 2n + 2m circulating lines (in each case n circulating lines for the different colors of unmodified water-borne base coats A and for the different colors of modified water-borne base coats modAB and in each case m circulating lines for the different colors of unmodified water-borne base coats B and for the different colors of modified water-borne base coats modB), but rather just n circulating lines for the different colors of unmodified water-borne base coats A plus m circulating lines for the different colors of unmodified water-borne base coats B plus one circulating line for the pigment-free admixture component.

In the process according to the invention, the EDC-primed substrates are initially spray-coated with the modified water-borne base coat modAB, preferably by electrostatically-assisted high-speed rotary atomization.

Then, preferably after a brief flash-off phase of, for example, 30 seconds to 5 minutes at an air temperature of 20 to 25°C, the corresponding unmodified water-borne base coat A is spray-applied, preferably by pneumatic spray application.

This is preferably also followed by a brief flash-off phase of, for example, 30 seconds to 10 minutes at an air temperature of 20 to 100°C, after which the clear coat is applied in a dry film thickness of, for example, 20 to 60 µm.

All known clear coats are in principle suitable as the clear coat. Usable clear coats are both solvent-containing one-component (1 pack) or two-component (2 pack) clear coats, water-dilutable 1 pack or 2 pack clear coats, powder clear coats or aqueous powder clear coat slurries. After an optional flash-off phase, the applied water-borne base coat layer consisting of modified water-borne base coat modAB and unmodified water-borne base coat A and the clear coat layer are jointly cured, for example, by baking, for example, at 80 to 160°C object temperature.

It is advantageous that repair coating of multi-layer coatings produced by the process according to the invention can be carried out with the unmodified water-borne base coat A of the relevant problematic color shade without there being any visually perceptible deviation in color shade in the area of the repair. In other words, consistency in color shade of the kind already mentioned above is ensured, even if the repair coating is performed using only the corresponding unmodified water-borne base coat A and not also the modified water-borne base coat modAB.

### Examples

### Example 1 (Production of a white unmodified water-borne base coat):

A white unmodified water-borne base coat of the following composition was produced:
17.2 pbw (parts by weight) of resin solids (7.8 pbw of a polyester acrylate resin, 5.9 pbw of a polyurethane resin, 3.5 pbw of hexamethoxymethylmelamine)
25.1 pbw of titanium dioxide (TiPure® R 706 from DuPont)
0.2 pbw of dimethylethanol amine
0.6 pbw of polyacrylic acid thickener
0.2 pbw of defoamer
1.0 pbw polypropylene glycol 900
45.1 pbw of deionized water
10.6 pbw of organic solvents (6.6 pbw of ethylene glycol monobutyl ether, 3.1 pbw of diethylene glycol monobutyl ether, 0.9 pbw of n-propanol).

### Example 2 (Production of a polyisocyanate admixture component):

A mixture of
30 pbw of N-methylpyrrolidone,
47 pbw of a hydrophilic aliphatic polyisocyanate based on hexamethylene diisocyanate with an NCO value of 17.4 and
23 pbw of a trimerized hexamethylene diisocyanate with an NCO value of 23
was produced.

### Example 3 (Production of water-borne base coats):

a) A yellow unmodified water-borne base coat of the following composition was produced:
   18.0 pbw of resin solids (8.1 pbw of a polyester acrylate resin, 6.2 pbw of a polyurethane resin, 3.7 pbw of hexamethoxymethylmelamine)
   0.4 pbw of Irgazin® Yellow 2RLT from Ciba
   2.9 pbw of titanium dioxide (TiPure® R 706 from DuPont)
   5.0 pbw of Irgacolor® Yellow 3GLM from Ciba
   4.2 pbw of Heucodur Yellow 3R from Heubach
   0.3 pbw of dimethylethanolamine
   0.2 pbw of defoamer
   0.6 pbw of polyacrylic acid thickener
   1.0 pbw of polypropylene glycol 900
   14.6 pbw of organic solvents (4.2 pbw of ethylene glycol monobutyl ether, 1.7 pbw of diethylene glycol monobutyl ether, 0.7 pbw of ethylene glycol monohexyl ether, 3.0 pbw of N-methylpyrrolidone, 3.5 pbw of n-butanol, 1.0 pbw of n-propanol, 0.5 pbw of Shellsol T)
   52.8 pbw of deionized water.
   The yellow unmodified water-borne base coat had a black/white opacity of 52 µm and a specific individual process film thickness of 15 µm.
b) A modified water-borne base coat was produced by mixing 100 pbw of the yellow unmodified water-borne base coat from a) with 400 pbw of the white unmodified water-borne base coat from Example 1 and with 50 pbw of the polyisocyanate admixture component from Example 2. The modified water-borne base coat had a specific individual process film thickness of 15 µm.
c) A water-borne coating composition was produced by mixing 100 pbw of the unmodified water-borne base coat from a) with 10 pbw of the polyisocyanate admixture component from Example 2.

### Examples 4a to 4c (Production of Multi-Layer Coatings):

4a) A multi-layer coating 4a was obtained by the following procedure:
   The modified water-borne base coat 3b was spray applied in a dry film thickness of 12 µm to automotive steel test panels 300 mm x 600 mm in size and provided with a dark-grey EDC primer (lightness L* = 8; colorimetrically determined at an illumination angle of 45° to the perpendicular and an observation angle of 45° relative to the specular. reflection).
   After flashing-off for 2 minutes at room temperature the yellow unmodified water-borne base coat 3a was spray applied in a wedge-shaped gradient (wedge in longitudinal direction) to a dry film thickness range from 0 to 20 µm and allowed to flash-off for 5 minutes at 80°C.
   The test panels provided in this way with a flashed off base coat layer were then spray coated with a commercial two-component polyurethane clear coat in a dry film thickness of 40 µm and after flashing-off for 5 minutes at 20°C baked for 20 minutes at 140°C object temperature.
4b): A multi-layer coating 4b was obtained by repeating Example 4a with the difference that the water-borne coating composition 3c was used instead of water-borne base coat 3b.
4c): A further multi-layer coating 4c was produced without making use of modified water-borne base coat 3b or water-borne coating composition 3c. To this end the yellow unmodified water-borne base coat 3a was spray applied in a dry film thickness of 60 µm to an automotive steel test panel provided with the dark-grey EDC primer. To this end 3 spray passes in each case followed by a forced drying step of 5 minutes at 70°C were performed. Thereafter the two-component polyurethane clear coat was spray applied in a dry film thickness of 40 µm and after flashing-off for 5 minutes at 20°C baked for 20 minutes at 140°C object temperature.

The multi-layer coatings 4a and 4b so obtained were in each case colorimetrically assessed at an illumination angle of 45° to the perpendicular and an observation angle of 45° relative to the specular reflection in accordance with the method known from US 5,991,042 using the X-Rite MA 68 II instrument sold by the company X-Rite. Multi-layer coating 4c was colorimetrically measured using the same equipment.

Table 1 shows the delta E values calculated from the colorimetric data as a function of the dry film thickness of the unmodified water-borne base coat 3a [delta E₄ₐ = square root of (L*_{4c}² - L*₄ₐ² + c*_{4c}² - c*₄ₐ² + h*_{4c}² -h*₄ₐ²); delta E_{4b} = square root of (L*_{4c}² - L*_{4b}² + c*_{4c}² - c*_{4b}² + h*_{4c}² - h*_{4b}²)].

**TABLE 1**

| Dry film thickness of 3a (µm) | 5 | 7 | 9 | 10 | 11 | 12 | 13 | 14 | 15 | 17 | 19 |
|---|---|---|---|---|---|---|---|---|---|---|---|
| delta E₄ₐ | 2.70 | 1.61 | 0.82 | 0.64 | 0.55 | 0.41 | 0.35 | 0.32 | 0.30 | 0.31 | 0.26 |
| delta E_{4b} | 5.01 | 4.81 | 4.68 | 4.42 | 4.31 | 4.14 | 3.99 | 3.76 | 3.56 | 3.43 | 3.18 |

## Claims

1. A process for the production of multi-layer coatings in A' color shades, comprising the successive steps:
1) applying a two-layered base coat layer in a total process film thickness in the range from 10 to 35 µm to a substrate provided with an EDC primer,
2) applying a clear coat layer onto the base coat layer,
3) jointly curing the base coat and clear coat layers,
wherein step 1) comprises (i) mixing 100 pbv of an unmodified water-borne base coat A having a color shade A' and having a black/white opacity of >25 µm and 1 to 400 pbv of an unmodified water-borne base coat B having a color shade B' to form an unmodified water-borne base coat AB, (ii) mixing the unmodified water-borne base coat AB with a pigment-free admixture component to form a modified water-borne base coat modAB, (iii) applying the first layer of the two-layered base coat layer from the modified water-borne base coat modAB and (iv) applying the second layer of the two-layered base coat layer from the unmodified water-borne base coat A,
wherein the pigment-free admixture component is a composition with a solids content of 20 to 95 wt.% consisting of a resin solids content plus possible nonvolatile additives, said resin solids content consisting of polyisocyanate(s),
wherein the admixture component is mixed into the unmodified water-borne base coat AB in a ratio by weight of 0.2 to 1 parts of polyisocyanate : 1 part of resin solids of the unmodified water-borne base coat AB, and
wherein the pigment content of the unmodified water-borne base coat B is made such that the multi-layer coating achieved after step 3) achieves color shade consistency from in each case at least 80% of the individual process film thickness both of the layer applied from the modified water-borne base coat modAB and of the layer applied from the unmodified water-borne base coat A.

2. The process of claim 1, wherein the individual process film thickness of the first base coat layer of the modified water-borne base coat modAB is in the range from 5 to 25 µm and the individual process film thickness of the second base coat layer of the unmodified water-borne base coat A is in the range from 3 to 20 µm.

3. The process of claim 1 or 2, wherein the unmodified water-borne base coat B has a solid color shade.

4. The process of claim 3, wherein the unmodified water-borne base coat A has a solid color shade.

5. The process of any one of the preceding claims being performed in an industrial coating facility.

6. The process of claim 5, wherein in addition substrates are provided with multi-layer coatings in B' color shades and wherein the unmodified water-borne base coats A and B together represent the color shade program selected for the substrates to be multi-layer coated.

7. The process of any one of the preceding claims, wherein the modified water-borne base coat modAB is applied by electrostatically-assisted high-speed rotary atomization and the unmodified water-borne base coat A is pneumatically spray-applied.

8. The process of any one of the preceding claims, wherein the substrate is selected from the group consisting of automotive bodies and automotive body parts.

## Patentansprüche

1. Verfahren für die Herstellung von mehrschichtigen Beschichtungen in A'-Farbschattierungen, umfassend die aufeinanderfolgenden Schritte:
1) das Aufbringen einer zweischichtigen Grundlackschicht in einer Gesamtprozessfilmdicke im Bereich von 10 bis 35 µm auf ein Substrat, das mit einer ETL-Grundierung versehen worden ist,
2) das Aufbringen einer Klarlackschicht auf die Grundlackschicht,
3) das gemeinsame Aushärten der Grundlack- und Klarlackschichten,
wobei der Schritt 1) Folgendes (i) umfasst: das Mischen von 100 Volumenteilen eines unmodifizierten Grundlacks A auf Wasserbasis, der eine Farbschattierung A' und eine Schwarz-Weiß-Opazität von >25 µm aufweist, und von 1 bis 400 Volumenteilen eines unmodifizierten Grundlacks B auf Wasserbasis, der eine Farbschattierung B' aufweist, um einen unmodifizierten Grundlack AB auf Wasserbasis zu bilden, (ii) das Mischen des unmodifizierten Grundlacks AB auf Wasserbasis mit einer pigmentfreien Mischungskomponente, um einen modifizierten Grundlack modAB auf Wasserbasis zu bilden, (iii) das Aufbringen der ersten Schicht der zweischichtigen Grundlackschicht aus dem modifizierten Grundlack modAB auf Wasserbasis und (iv) das Aufbringen der zweiten Schicht der zweischichtigen Grundlackschicht aus dem unmodifizierten Grundlack A auf Wasserbasis,
wobei die pigmentfreie Mischungskomponente eine Zusammensetzung mit einem Feststoffgehalt von 20 bis 95 Gew.-% ist, der aus einem Harzfeststoffgehalt plus möglichen nichtflüchtigen Zusatzmitteln besteht, wobei der Harzfeststoffgehalt aus Polyisocyanat(en) besteht,
wobei die Mischungskomponente in den unmodifizierten Grundlack AB auf Wasserbasis in einem Gewichtsverhältnis von 0,2 bis 1 Teile Polyisocyanat : 1 Teil Harzfeststoffe des unmodifizierten Grundlacks AB auf Wasserbasis gemischt wird und
wobei der Pigmentgehalt des unmodifizierten Grundlacks B auf Wasserbasis derart hergestellt ist, dass die mehrschichtige Beschichtung, die nach Schritt 3) erreicht wird, eine Farbschattierungskonsistenz von, in jedem Fall, mindestens 80 % der einzelnen Prozessfilmdicken sowohl der Schicht, die aus dem modifizierten Grundlack modAB auf Wasserbasis aufgebracht wird, als auch der Schicht, die aus dem unmodifizierten Grundlack A auf Wasserbasis aufgebracht wird, erreicht.

2. Verfahren nach Anspruch 1, wobei die einzelne Prozessfilmdicke der ersten Grundlackschicht aus dem modifizierten Grundlack modAB auf Wasserbasis im Bereich von 5 bis 25 µm liegt und die einzelne Prozessfilmdicke der zweiten Grundlackschicht aus dem unmodifizierten Grundlack A auf Wasserbasis im Bereich von 3 bis 20 µm liegt.

3. Verfahren nach Anspruch 1 oder 2, wobei der unmodifizierte Grundlack B auf Wasserbasis eine massive Farbschattierung aufweist.

4. Verfahren nach Anspruch 3, wobei der unmodifizierte Grundlack A auf Wasserbasis eine massive Farbschattierung aufweist.

5. Verfahren nach einem der vorhergehenden Ansprüche, das in einer technischen Beschichtungsanlage durchgeführt wird.

6. Verfahren nach Anspruch 5, wobei zusätzlich Substrate mit mehrschichtigen Beschichtungen in B'-Farbschattierungen versehen werden und wobei die unmodifizierten Grundlacke A und B auf Wasserbasis zusammen das Farbschattierungsprogramm darstellen, das ausgewählt wird, damit die Substrate mehrschichtig beschichtet werden.

7. Verfahren nach einem der vorhergehenden Ansprüche, wobei der modifizierte Grundlack modAB auf Wasserbasis durch elektrostatisch unterstützte Hochgeschwindigkeitsrotationsatomisierung aufgebracht wird und der unmodifizierte Grundlack A auf Wasserbasis durch pneumatisches Spritzen aufgebracht wird.

8. Verfahren nach einem der vorhergehenden Ansprüche, wobei das Substrat aus der Gruppe ausgewählt wird bestehend aus Fahrzeugkarosserien und Fahrzeugkarosserieteilen.

## Revendications

1. Procédé de production de revêtements multicouches dans des teintes A', comprenant les étapes successives consistant à :
1) appliquer une couche de revêtement de base bicouche selon une épaisseur de film du procédé totale comprise dans la plage allant de 10 à 35 µm sur un substrat pourvu d'une amorce EDC,
2) appliquer une couche de revêtement transparent sur la couche de revêtement de base,
3) durcir conjointement la couche de revêtement de base et la couche de revêtement transparent,
dans lequel l'étape 1) consiste à (i) mélanger 100 pbv d'un revêtement de base à base d'eau non modifié A ayant une teinte A' et ayant une opacité noir/blanc > 25 µm et de 1 à 400 pbv d'un revêtement de base à base d'eau non modifié B ayant une teinte B' pour former un revêtement de base à base d'eau non modifié AB, (ii) mélanger le revêtement de base à base d'eau non modifié AB avec un composant de mélange sans pigment pour former un revêtement de base à base d'eau modifié modAB, (iii) appliquer la première couche de la couche de revêtement de base bicouche provenant du revêtement de base à base d'eau modifié modAB et (iv) appliquer la seconde couche de la couche de revêtement de base bicouche provenant du revêtement de base à base d'eau non modifié A,
dans lequel le composant de mélange sans pigment est une composition ayant une teneur en matières solides de 20 à 95 % en poids se composant d'une teneur en matières solides résineuses et éventuellement d'additifs non volatils, ladite teneur en matières solides résineuses se composant de polyisocyanate(s),
dans lequel le composant de mélange est mélangé dans le revêtement de base à base d'eau non modifié AB selon un rapport en poids de 0,2 à 1 partie de polyisocyanate:1 partie de matières solides résineuses du revêtement de base à base d'eau non modifié AB, et
dans lequel la teneur en pigment du revêtement de base à base d'eau non modifié B est telle que le revêtement multicouche obtenu après l'étape 3) atteint une consistante de teinte, dans chaque cas, d'au moins 80 % de l'épaisseur de film du procédé individuelle à la fois de la couche appliquée à partir du revêtement de base à base d'eau modifié modAB et de la couche appliquée à partir du revêtement de base à base d'eau non modifié A.

2. Procédé selon la revendication 1, dans lequel l'épaisseur de film du procédé individuelle de la première couche de revêtement de base du revêtement de base à base d'eau modifié modAB est comprise dans la plage allant de 5 à 25 µm et l'épaisseur de film du procédé individuelle de la seconde couche de revêtement de base du revêtement de base à base d'eau non modifié A est comprise dans la plage allant de 3 à 20 µm.

3. Procédé selon la revendication 1 ou 2, dans lequel le revêtement de base à base d'eau non modifié B a une teinte en aplat.

4. Procédé selon la revendication 3, dans lequel le revêtement de base à base d'eau non modifié A a une teinte en aplat.

5. Procédé selon l'une quelconque des revendications précédentes, qui est réalisé dans une installation de revêtement industrielle.

6. Procédé selon la revendication 5, dans lequel en outre des substrats sont fournis avec des revêtements multicouches dans des teintes B' et dans lequel les revêtements de base à base d'eau non modifiés A et B représentent ensemble le programme de teinte choisi pour les substrats à revêtir de plusieurs couches.

7. Procédé selon l'une quelconque des revendications précédentes, dans lequel le revêtement de base à base d'eau modifié modAB est appliqué par atomisation rotative à grande vitesse électrostatistiquement assistée et le revêtement de base à base d'eau non modifié A est appliqué par atomisation pneumatique.

8. Procédé selon l'une quelconque des revendications précédentes, dans lequel le substrat est choisi dans le groupe constitué par les corps automobiles et les parties de corps automobiles.
